# EUROPEAN PATENT SPECIFICATION

(11) **EP 3 456 421 B1**
(45) Date of publication and mention of the grant of the patent: **12.10.2022**
(21) Application number: 18194135.2
(22) Date of filing: 12.09.2018
(51) Int. Cl.: B05D 3/12, B05D 7/14, B05D 7/00, B05D 5/06, B05D 1/02, B05D 1/06, B05D 3/02

(54) **METHOD FOR COLOR-REGISTER SPRAYING OF HUB**
VERFAHREN ZUM FARBREGISTERSPRITZEN EINER NABE
PROCÉDÉ DE PULVÉRISATION DE MOYEN PAR REGISTRE DE COULEUR

(30) Priority: 13.09.2017 CN 201710822696
(43) Date of publication of application: 20.03.2019
(73) Proprietor: CITIC Dicastal Co., Ltd, Qinhuangdao Heibei 066011 (CN)
(72) Inventor: ZHAO, Qun, Qinhuangdao, Heibei 066011 (CN); BAO, Lei, Qinhuangdao, Heibei 066011 (CN); WANG, Le, Qinhuangdao, Heibei 066011 (CN); CHEN, Guangcai, Qinhuangdao, Heibei 066011 (CN); ZHANG, Shengchao, Qinhuangdao, Heibei 066011 (CN)
(74) Representative: Gong, Jinping

(56) References cited:
- WO-A1-2007/040284
- WO-A1-2013/023419
- FR-A1- 2 983 120
- US-A1- 2005 241 950
- US-A1- 2006 019 089
- US-A1- 2006 188 652
- US-A1- 2013 071 576

## Description

### Field of the Invention

The present invention relates to the manufacturing field of automobile parts, and s pecifically, relates to a method for color-register spraying of a hub.

### Background of the Invention

At present, the hub is relatively single in color. The existing color-register process is mainly achieved by protection, but has the problems that the color-register edge is not clear and needs to be partially repaired by manual operation, the yield is low, the labor cost is high and the like, so it is not suitable for batch production.

WO 2013/023419 A1 relates to an improved wheel coating process.

FR 2 983 120 A1 concerns a method of obtaining a wheel to be painted.

US 2005/241950 A1 relates to a method for forming a coating on a wheel.

WO 2007/040284 A1 provides a photoluminescent coating light alloy wheel.

### Summary of the Invention

Accordingly, the objective of the present invention is to provide a hub printing method which is simple in process and clear in color-register edge.

In one aspect of the present invention, provided is a method for color-register spraying of a hub as specified in any of claims 1 to 8. The method is characterized by comprising: after a black paint is sprayed onto the surface of the hub, machining a turned glossy surface, and then spraying the hub with a color celluloid paint.

In a preferred aspect of the present invention, the method comprises the steps of: pretreating→drying→spraying base powder→curing→spraying a black paint→curing→ machining a turned glossy surface→pretreating→drying→spraying transparent powder→ curing→spraying a color celluloid paint→curing.

In a preferred aspect of the present invention, the method adopts one or more of the following working conditions: (1) in the process of spraying base powder, an electrostatic spray gun is adopted for spraying, the voltage is controlled at 60~80 KV, and the powder output is controlled at 10~15 g/s, thereby ensuring excellent adhesion between coatings; (2) in the process of curing the base powder, the surface temperature of a workpiece is controlled at 180°C for 8~12 min, so that the powder maintains certain flexibility and better coating adhesion; (3) in the process of spraying a black paint, an air spray gun is adopted for spraying, the air output is controlled at 50~100 cc/min, and the atomizing sector pressure is 2~3 bar, so that the black paint is uniformly and fully sprayed on the surface of the hub; (4) in the process of curing the black paint, the temperature of the workpiece is controlled at 150°C for 10~15 min, so that the black paint has good flexibility and coating adhesion;
(5) in the process of machining a turned glossy surface, the revolving speed S is controlled at 1200 rpm, and the feed rate F is 0.2 mm/r; (6) in the process of spraying transparent powder, the electrostatic spray gun is adopted for spraying, the voltage is controlled at 60-80 KV, and the powder output is controlled at 10-15 g/s, thereby ensuring excellent adhesion between coatings; (7) in the process of curing the transparent powder, the surface temperature of the workpiece is controlled at 177°C for 10-15 min, so that the powder maintains certain flexibility and better coating adhesion; (8) in the process of spraying a color celluloid paint, a rotary cup spray gun is adopted for spraying, the revolving speed is 25000 R/min, the forming gas is 2-3 bar, and the paint output pressure is 4-5 bar, thereby ensuring that the color celluloid paint is uniformly and fully sprayed on the surface of the hub; and (9) in the process of curing the color celluloid paint, the temperature of the workpiece is controlled at 150°C for 10-15 min, so that the color celluloid paint has better flexibility and coating adhesion.

In a preferred aspect of the present invention, in the process of spraying base powder, an electrostatic spray gun is adopted for spraying, the voltage is controlled at 60 KV, and the powder output is controlled at 10 g/s, thereby ensuring excellent adhesion between coatings; in the process of curing the base powder, the surface temperature of a workpiece is controlled at 180°C for 8 min, so that the powder maintains certain flexibility and better coating adhesion; in the process of spraying a black paint, an air spray gun is adopted for spraying, the air output is controlled at 50 cc/min, and the atomizing sector pressure is 2 bar, so that the black paint is uniformly and fully sprayed on the surface of the hub; in the process of curing the black paint, the temperature of the workpiece is controlled at 150°C for 10 min, so that the black paint has good flexibility and coating adhesion; in the process of machining a turned glossy surface, the revolving speed S is controlled at 1200 rpm, and the feed rate F is 0.2 mm/r; in the process of spraying transparent powder, the electrostatic spray gun is adopted for spraying, the voltage is controlled at 60 KV, and the powder output is controlled at 10 g/s, thereby ensuring excellent adhesion between coatings; in the process of curing the transparent powder, the surface temperature of the workpiece is controlled at 177°C for 8 min, so that the powder maintains certain flexibility and better coating adhesion; in the process of spraying a color celluloid paint, a rotary cup spray gun is adopted for spraying, and the revolving speed is 25000 R/min; and in the process of curing the color celluloid paint, the temperature of the workpiece is controlled at 150°C for 10 min, so that the color celluloid paint has better flexibility and coating adhesion.

In a preferred aspect of the present invention, in the process of spraying base powder, an electrostatic spray gun is adopted for spraying, the voltage is controlled at 70 KV, and the powder output is controlled at 12 g/s, thereby ensuring excellent adhesion between coatings; in the process of curing the base powder, the surface temperature of a workpiece is controlled at 180°C for 10 min, so that the powder maintains certain flexibility and better coating adhesion; in the process of spraying a black paint, an air spray gun is adopted for spraying, the air output is controlled at 80 cc/min, and the atomizing sector pressure is 2.5 bar, so that the black paint is uniformly and fully sprayed on the surface of the hub; in the process of curing the black paint, the temperature of the workpiece is controlled at 150°C for 12 min, so that the black paint has good flexibility and coating adhesion; in the process of machining a turned glossy surface, the revolving speed S is controlled at 1200 rpm, and the feed rate F is 0.2 mm/r; in the process of spraying transparent powder, the electrostatic spray gun is adopted for spraying, the voltage is controlled at 70 KV, and the powder output is controlled at 12 g/s, thereby ensuring excellent adhesion between coatings; in the process of curing the transparent powder, the surface temperature of the workpiece is controlled at 177°C for 12 min, so that the powder maintains certain flexibility and better coating adhesion; in the process of spraying a color celluloid paint, a rotary cup spray gun is adopted for spraying, the revolving speed is 25000 R/min, the forming gas is 2.5 bar, and the paint output pressure is 4.5 bar, thereby ensuring that the color celluloid paint is uniformly and fully sprayed on the surface of the hub; and in the process of curing the color celluloid paint, the temperature of the workpiece is controlled at 150°C for 12 min, so that the color celluloid paint has better flexibility and coating adhesion.

In a preferred aspect of the present invention, in the process of spraying base powder, an electrostatic spray gun is adopted for spraying, the voltage is controlled at 80 KV, and the powder output is controlled at 15 g/s, thereby ensuring excellent adhesion between coatings; in the process of curing the base powder, the surface temperature of a workpiece is controlled at 180°C for 12 min, so that the powder maintains certain flexibility and better coating adhesion; in the process of spraying a black paint, an air spray gun is adopted for spraying, the air output is controlled at 100 cc/min, and the atomizing sector pressure is 3 bar, so that the black paint is uniformly and fully sprayed on the surface of the hub; in the process of curing the black paint, the temperature of the workpiece is controlled at 150°C for 15 min, so that the black paint has good flexibility and coating adhesion; in the process of machining a turned glossy surface, the revolving speed S is controlled at 1200 rpm, and the feed rate F is 0.2 mm/r; in the process of spraying transparent powder, the electrostatic spray gun is adopted for spraying, the voltage is controlled at 80 KV, and the powder output is controlled at 15 g/s, thereby ensuring excellent adhesion between coatings; in the process of curing the transparent powder, the surface temperature of the workpiece is controlled at 177°C for 15 min, so that the powder maintains certain flexibility and better coating adhesion; in the process of spraying a color celluloid paint, a rotary cup spray gun is adopted for spraying, the revolving speed is 25000 R/min, the forming gas is 3 bar, and the paint output pressure is 5 bar, thereby ensuring that the color celluloid paint is uniformly and fully sprayed on the surface of the hub; and in the process of curing the color celluloid paint, the temperature of the workpiece is controlled at 150°C for 15 min, so that the color celluloid paint has better flexibility and coating adhesion.

In other aspect of the present invention, further disclosed is the following technical solution:
In order to solve the technological deficiencies of color registration of the hub, the present invention provides a novel hub color-register spraying process.

The specific process flow of the present invention is: pretreating→drying →spraying base powder→ curing →spraying a black paint-curing-machining a turned glossy surface→pretreating→drying →spraying transparent powder→curing→spraying a color celluloid paint→curing.

In the process of spraying base powder, an electrostatic spray gun is adopted for spraying, the voltage is controlled at 60-80 KV, and the powder output is controlled at 10-15 g/s, thereby ensuring excellent adhesion between coatings.

In the process of curing the base powder, the surface temperature of a workpiece is controlled at 180°C for 8-12 min, so that the powder maintains certain flexibility and better coating adhesion.

In the process of spraying a black paint, an air spray gun is adopted for spraying, the air output is controlled at 50-100 cc/min, and the atomizing sector pressure is 2-3 bar, thereby ensuring that the black paint is uniformly and fully sprayed on the surface of the hub.

In the process of curing the black paint, the temperature of the workpiece is controlled at 150°C for 10~15 min, so that the black paint has good flexibility and coating adhesion.

In the process of machining a turned glossy surface, the revolving speed S is controlled at 1200 rpm, and the feed rate F is 0.2 mm/r.

In the process of spraying transparent powder, the electrostatic spray gun is adopted for spraying, the voltage is controlled at 60-80 KV, and the powder output is controlled at 10-15 g/s, thereby ensuring excellent adhesion between coatings.

In the process of curing the transparent powder, the surface temperature of the workpiece is controlled at 177°C for 10-15 min, so that the powder maintains certain flexibility and better coating adhesion.

In the process of spraying a color celluloid paint, a rotary cup spray gun is adopted for spraying, the revolving speed is 25000 R/min, the forming gas is 2-3 bar, and the paint output pressure is 4-5 bar, thereby ensuring that the color celluloid paint is uniformly and fully sprayed on the surface of the hub.

In the process of curing the color celluloid paint, the temperature of the workpiece is controlled at 150°C for 10-15 min, so that the color celluloid paint has better flexibility and coating adhesion. The present invention achieves a color-register spraying effect by spraying the color celluloid paint, greatly improves the production efficiency, and can achieve batch production.

In a preferred aspect, in the process of spraying base powder, an electrostatic spray gun is adopted for spraying, the voltage is controlled at 60 KV, and the powder output is controlled at 10 g/s, thereby ensuring excellent adhesion between coatings. In the process of curing the base powder, the surface temperature of a workpiece is controlled at 180°C for 8 min, so that the powder maintains certain flexibility and better coating adhesion. In the process of spraying a black paint, an air spray gun is adopted for spraying, the air output is controlled at 50 cc/min, and the atomizing sector pressure is 2 bar, thereby ensuring that the black paint is uniformly and fully sprayed on the surface of the hub. In the process of curing the black paint, the temperature of the workpiece is controlled at 150°C for 10 min, so that the black paint has good flexibility and coating adhesion. In the process of machining a turned glossy surface, the revolving speed S is controlled at 1200 rpm, and the feed rate F is 0.2 mm/r. In the process of spraying transparent powder, the electrostatic spray gun is adopted for spraying, the voltage is controlled at 60 KV, and the powder output is controlled at 10 g/s, thereby ensuring excellent adhesion between coatings. In the process of curing the transparent powder, the surface temperature of the workpiece is controlled at 177°C for 8 min, so that the powder maintains certain flexibility and better coating adhesion. In the process of spraying a color celluloid paint, a rotary cup spray gun is adopted for spraying, the revolving speed is 25000 R/min, the forming gas is 2 bar, and the paint output pressure is 4 bar, thereby ensuring that the color celluloid paint is uniformly and fully sprayed on the surface of the hub. In the process of curing the color celluloid paint, the temperature of the workpiece is controlled at 150°C for 10 min, so that the color celluloid paint has better flexibility and coating adhesion.

In a preferred aspect, in the process of spraying base powder, an electrostatic spray gun is adopted for spraying, the voltage is controlled at 70 KV, and the powder output is controlled at 12g/s, thereby ensuring excellent adhesion between coatings. In the process of curing the base powder, the surface temperature of a workpiece is controlled at 180°C for 10 min, so that the powder maintains certain flexibility and better coating adhesion. In the process of spraying a black paint, an air spray gun is adopted for spraying, the air output is controlled at 80 cc/min, and the atomizing sector pressure is 2.5 bar, thereby ensuring that the black paint is uniformly and fully sprayed on the surface of the hub. In the process of curing the black paint, the temperature of the workpiece is controlled at 150°C for 12 min, so that the black paint has good flexibility and coating adhesion. In the process of machining a turned glossy surface, the revolving speed S is controlled at 1200 rpm, and the feed rate F is 0.2 mm/r. In the process of spraying transparent powder, the electrostatic spray gun is adopted for spraying, the voltage is controlled at 70KV, and the powder output is controlled at 12g/s, thereby ensuring excellent adhesion between coatings. In the process of curing the transparent powder, the surface temperature of the workpiece is controlled at 177°C for 12 min, so that the powder maintains certain flexibility and better coating adhesion. In the process of spraying a color celluloid paint, a rotary cup spray gun is adopted for spraying, the revolving speed is 25000 R/min, the forming gas is 2.5 bar, and the paint output pressure is 4.5 bar, thereby ensuring that the color celluloid paint is uniformly and fully sprayed on the surface of the hub. In the process of curing the color celluloid paint, the temperature of the workpiece is controlled at 150°C for 12 min, so that the color celluloid paint has better flexibility and coating adhesion.

In a preferred aspect, in the process of spraying base powder, an electrostatic spray gun is adopted for spraying, the voltage is controlled at 80 KV, and the powder output is controlled at 15 g/s, thereby ensuring excellent adhesion between coatings. In the process of curing the base powder, the surface temperature of a workpiece is controlled at 180°C for 12 min, so that the powder maintains certain flexibility and better coating adhesion. In the process of spraying a black paint, an air spray gun is adopted for spraying, the air output is controlled at 100 cc/min, and the atomizing sector pressure is 3 bar, thereby ensuring that the black paint is uniformly and fully sprayed on the surface of the hub. In the process of curing the black paint, the temperature of the workpiece is controlled at 150°C for 15 min, so that the black paint has good flexibility and coating adhesion. In the process of machining a turned glossy surface, the revolving speed S is controlled at 1200 rpm, and the feed rate F is 0.2 mm/r. In the process of spraying transparent powder, the electrostatic spray gun is adopted for spraying, the voltage is controlled at 80 KV, and the powder output is controlled at 15 g/s, thereby ensuring excellent adhesion between coatings. In the process of curing the transparent powder, the surface temperature of the workpiece is controlled at 177°C for 15 min, so that the powder maintains certain flexibility and better coating adhesion. In the process of spraying a color celluloid paint, a rotary cup spray gun is adopted for spraying, the revolving speed is 25000 R/min, the forming gas is 3 bar, and the paint output pressure is 5 bar, thereby ensuring that the color celluloid paint is uniformly and fully sprayed on the surface of the hub. In the process of curing the color celluloid paint, the temperature of the workpiece is controlled at 150°C for 15 min, so that the color celluloid paint has better flexibility and coating adhesion.

The present invention achieves a color-register spraying effect by spraying the color celluloid paint, greatly improves the production efficiency, and can achieve batch production.

### Detailed Description of the Embodiments

### Embodiment 1

The specific process flow of a color celluloid paint color-register spraying process is: pretreating→ drying-spraying base powder→curing→spraying a black paint→curing→machining a turned glossy surface→pretreating→drying→spraying transparent powder→curing→spraying a color celluloid paint→curing.

In the process of spraying base powder, an electrostatic spray gun is adopted for spraying, the voltage is controlled at 60 KV, and the powder output is controlled at 10 g/s, thereby ensuring excellent adhesion between coatings.

In the process of curing the base powder, the surface temperature of a workpiece is controlled at 180°C for 8 min, so that the powder maintains certain flexibility and better coating adhesion.

In the process of spraying a black paint, an air spray gun is adopted for spraying, the air output is controlled at 50 cc/min, and the atomizing sector pressure is 2 bar, thereby ensuring that the black paint is uniformly and fully sprayed on the surface of the hub.

In the process of curing the black paint, the temperature of the workpiece is controlled at 150°C for 10 min, so that the black paint has good flexibility and coating adhesion.

In the process of machining a turned glossy surface, the revolving speed S is controlled at 1200 rpm, and the feed rate F is 0.2 mm/r.

In the process of spraying transparent powder, the electrostatic spray gun is adopted for spraying, the voltage is controlled at 60 KV, and the powder output is controlled at 10 g/s, thereby ensuring excellent adhesion between coatings.

In the process of curing the transparent powder, the surface temperature of the workpiece is controlled at 177°C for 8 min, so that the powder maintains certain flexibility and better coating adhesion.

In the process of spraying a color celluloid paint, a rotary cup spray gun is adopted for spraying, and the revolving speed is 25000 R/min.

In the process of curing the color celluloid paint, the temperature of the workpiece is controlled at 150°C for 10min, so that the color celluloid paint has better flexibility and coating adhesion.

### Embodiment 2

The specific process flow of a color celluloid paint color-register spraying process is: pretreating→ drying-spraying base powder→curing→spraying a black paint→curing→machining a turned glossy surface→pretreating→drying→spraying transparent powder→curing→spraying a color celluloid paint→curing.

In the process of spraying base powder, an electrostatic spray gun is adopted for spraying, the voltage is controlled at 70KV, and the powder output is controlled at 12 g/s, thereby ensuring excellent adhesion between coatings.

In the process of curing the base powder, the surface temperature of a workpiece is controlled at 180°C for 10 min, so that the powder maintains certain flexibility and better coating adhesion.

In the process of spraying a black paint, an air spray gun is adopted for spraying, the air output is controlled at 80 cc/min, and the atomizing sector pressure is 2.5 bar, thereby ensuring that the black paint is uniformly and fully sprayed on the surface of the hub.

In the process of curing the black paint, the temperature of the workpiece is controlled at 150°C for 12 min, so that the black paint has good flexibility and coating adhesion.

In the process of machining a turned glossy surface, the revolving speed S is controlled at 1200 rpm, and the feed rate F is 0.2 mm/r.

In the process of spraying transparent powder, the electrostatic spray gun is adopted for spraying, the voltage is controlled at 70 KV, and the powder output is controlled at 12 g/s, thereby ensuring excellent adhesion between coatings.

In the process of curing the transparent powder, the surface temperature of the workpiece is controlled at 177°C for 12 min, so that the powder maintains certain flexibility and better coating adhesion.

In the process of spraying a color celluloid paint, a rotary cup spray gun is adopted for spraying, the revolving speed is 25000 R/min, the forming gas is 2.5 bar, and the paint output pressure is 4.5 bar, thereby ensuring that the color celluloid paint is uniformly and fully sprayed on the surface of the hub.

In the process of curing the color celluloid paint, the temperature of the workpiece is controlled at 150°C for 12 min, so that the color celluloid paint has better flexibility and coating adhesion.

### Embodiment 3

The specific process flow of a color celluloid paint color-register spraying process is: pretreating→ drying-spraying base powder→curing→spraying a black paint→curing→machining a turned glossy surface→pretreating→drying→spraying transparent powder→curing→spraying a color celluloid paint→curing.

In the process of spraying base powder, an electrostatic spray gun is adopted for spraying, the voltage is controlled at 80 KV, and the powder output is controlled at 15 g/s, thereby ensuring excellent adhesion between coatings.

In the process of curing the base powder, the surface temperature of a workpiece is controlled at 180°C for 12 min, so that the powder maintains certain flexibility and better coating adhesion.

In the process of spraying a black paint, an air spray gun is adopted for spraying, the air output is controlled at 100 cc/min, and the atomizing sector pressure is 3 bar, thereby ensuring that the black paint is uniformly and fully sprayed on the surface of the hub.

In the process of curing the black paint, the temperature of the workpiece is controlled at 150°C for 15 min, so that the black paint has good flexibility and coating adhesion.

In the process of machining a turned glossy surface, the revolving speed S is controlled at 1200 rpm, and the feed rate F is 0.2 mm/r.

In the process of spraying transparent powder, the electrostatic spray gun is adopted for spraying, the voltage is controlled at 80 KV, and the powder output is controlled at 15 g/s, thereby ensuring excellent adhesion between coatings.

In the process of curing the transparent powder, the surface temperature of the workpiece is controlled at 177°C for 15 min, so that the powder maintains certain flexibility and better coating adhesion.

In the process of spraying a color celluloid paint, a rotary cup spray gun is adopted for spraying, the revolving speed is 25000 R/min, the forming gas is 3 bar, and the paint output pressure is 5 bar, thereby ensuring that the color celluloid paint is uniformly and fully sprayed on the surface of the hub.

In the process of curing the color celluloid paint, the temperature of the workpiece is controlled at 150°C for 15 min, so that the color celluloid paint has better flexibility and coating adhesion.

## Claims

1. A method for color-register spraying of a hub, comprising: after a black paint is sprayed onto the surface of the hub, machining a turned glossy surface, and then spraying the hub with a color celluloid paint,
wherein the method comprises the steps of: pretreating→drying→spraying base powder→ curing→spraying a black paint→curing→machining a turned glossy surface→pretreating→ drying→spraying transparent powder→curing→spraying a color celluloid paint→curing,
wherein in the process of spraying a color celluloid paint, a rotary cup spray gun is adopted for spraying, the revolving speed is 25000 R/min, the forming gas is 2~3 bar, and the paint output pressure is 4~5 bar, thereby ensuring that the color celluloid paint is uniformly and fully sprayed on the surface of the hub; and
wherein in the process of curing the color celluloid paint, the temperature of the workpiece is controlled at 150°C for 10~15 min, so that the color celluloid paint has better flexibility and coating adhesion.

2. The method according to claim 1, wherein (1) in the process of spraying base powder, an electrostatic spray gun is adopted for spraying, the voltage is controlled at 60~80 KV, and the powder output is controlled at 10~15 g/s, thereby ensuring excellent adhesion between coatings; and/or
(2) in the process of curing the base powder, the surface temperature of a workpiece is controlled at 180°C for 8~12 min, so that the powder maintains certain flexibility and better coating adhesion.

3. The method according to claim 1 or 2, wherein in the process of spraying a black paint, an air spray gun is adopted for spraying, the air output is controlled at 50~100 cc/min, and the atomizing sector pressure is 2~3 bar, thereby ensuring that the black paint is uniformly and fully sprayed on the surface of the hub; and/or
in the process of curing the black paint, the temperature of the workpiece is controlled at 150°C for 10~15 min, so that the black paint has good flexibility and coating adhesion.

4. The method according to one of claims 1 to 3, wherein in the process of machining a turned glossy surface, the revolving speed S is controlled at 1200 rpm, and the feed rate F is 0.2 mm/r.

5. The method according to one of claims 1 to 4, wherein in the process of spraying transparent powder, the electrostatic spray gun is adopted for spraying, the voltage is controlled at 60~80 KV, and the powder output is controlled at 10~15 g/s, thereby ensuring excellent adhesion between coatings; and/or
in the process of curing the transparent powder, the surface temperature of the workpiece is controlled at 177°C for 10~15 min, so that the powder maintains certain flexibility and better coating adhesion.

6. The method according to one of claims 1 to 5, wherein,
in the process of spraying base powder, an electrostatic spray gun is adopted for spraying, the voltage is controlled at 60 KV, and the powder output is controlled at 10 g/s, thereby ensuring excellent adhesion between coatings;
in the process of curing the base powder, the surface temperature of a workpiece is controlled at 180°C for 8 min, so that the powder maintains certain flexibility and better coating adhesion;
in the process of spraying a black paint, an air spray gun is adopted for spraying, the air output is controlled at 50 cc/min, and the atomizing sector pressure is 2 bar, thereby ensuring that the black paint is uniformly and fully sprayed on the surface of the hub;
in the process of curing the black paint, the temperature of the workpiece is controlled at 150°C for 10 min, so that the black paint has good flexibility and coating adhesion;
in the process of machining a turned glossy surface, the revolving speed S is controlled at 1200 rpm, and the feed rate F is 0.2 mm/r;
in the process of spraying transparent powder, the electrostatic spray gun is adopted for spraying, the voltage is controlled at 60 KV, and the powder output is controlled at 10 g/s, thereby ensuring excellent adhesion between coatings;
in the process of curing the transparent powder, the surface temperature of the workpiece is controlled at 177°C for 8 min, so that the powder maintains certain flexibility and better coating adhesion;
in the process of spraying a color celluloid paint, a rotary cup spray gun is adopted for spraying, and the revolving speed is 25000 R/min; and
in the process of curing the color celluloid paint, the temperature of the workpiece is controlled at 150°C for 10 min, so that the color celluloid paint has better flexibility and coating adhesion.

7. The method according to one of claims 1 to 5, wherein,
in the process of spraying base powder, an electrostatic spray gun is adopted for spraying, the voltage is controlled at 70 KV, and the powder output is controlled at 12 g/s, thereby ensuring excellent adhesion between coatings;
in the process of curing the base powder, the surface temperature of a workpiece is controlled at 180°C for 10 min, so that the powder maintains certain flexibility and better coating adhesion;
in the process of spraying a black paint, an air spray gun is adopted for spraying, the air output is controlled at 80 cc/min, and the atomizing sector pressure is 2.5 bar, thereby ensuring that the black paint is uniformly and fully sprayed on the surface of the hub;
in the process of curing the black paint, the temperature of the workpiece is controlled at 150°C for 12 min, so that the black paint has good flexibility and coating adhesion;
in the process of machining a turned glossy surface, the revolving speed S is controlled at 1200 rpm, and the feed rate F is 0.2 mm/r;
in the process of spraying transparent powder, the electrostatic spray gun is adopted for spraying, the voltage is controlled at 70 KV, and the powder output is controlled at 12 g/s, thereby ensuring excellent adhesion between coatings;
in the process of curing the transparent powder, the surface temperature of the workpiece is controlled at 177°C for 12 min, so that the powder maintains certain flexibility and better coating adhesion;
in the process of spraying a color celluloid paint, a rotary cup spray gun is adopted for spraying, the revolving speed is 25000 R/min, the forming gas is 2.5 bar, and the paint output pressure is 4.5 bar, thereby ensuring that the color celluloid paint is uniformly and fully sprayed on the surface of the hub; and
in the process of curing the color celluloid paint, the temperature of the workpiece is controlled at 150°C for 12 min, so that the color celluloid paint has better flexibility and coating adhesion.

8. The method according to one of claims 1 to 5, wherein,
in the process of spraying base powder, an electrostatic spray gun is adopted for spraying, the voltage is controlled at 80 KV, and the powder output is controlled at 15 g/s, thereby ensuring excellent adhesion between coatings;
in the process of curing the base powder, the surface temperature of a workpiece is controlled at 180°C for 12 min, so that the powder maintains certain flexibility and better coating adhesion;
in the process of spraying a black paint, an air spray gun is adopted for spraying, the air output is controlled at 100 cc/min, and the atomizing sector pressure is 3 bar, thereby ensuring that the black paint is uniformly and fully sprayed on the surface of the hub;
in the process of curing the black paint, the temperature of the workpiece is controlled at 150°C for 15min, so that the black paint has good flexibility and coating adhesion;
in the process of machining a turned glossy surface, the revolving speed S is controlled at 1200 rpm, and the feed rate F is 0.2 mm/r;
in the process of spraying transparent powder, the electrostatic spray gun is adopted for spraying, the voltage is controlled at 80 KV, and the powder output is controlled at 15 g/s, thereby ensuring excellent adhesion between coatings;
in the process of curing the transparent powder, the surface temperature of the workpiece is controlled at 177°C for 15 min, so that the powder maintains certain flexibility and better coating adhesion;
in the process of spraying a color celluloid paint, a rotary cup spray gun is adopted for spraying, the revolving speed is 25000 R/min, the forming gas is 3 bar, and the paint output pressure is 5 bar, thereby ensuring that the color celluloid paint is uniformly and fully sprayed on the surface of the hub; and
in the process of curing the color celluloid paint, the temperature of the workpiece is controlled at 150°C for 15 min, so that the color celluloid paint has better flexibility and coating adhesion.

## Patentansprüche

1. Verfahren zum Farbregistersprühen einer Nabe, umfassend: nachdem eine schwarze Farbe auf die Oberfläche der Nabe gesprüht wurde, Bearbeiten einer gedrehten glänzenden Oberfläche und dann Besprühen der Nabe mit einer farbigen Zelluloidfarbe,
wobei das Verfahren die Schritte umfasst: Vorbehandeln→Trocknen→Sprühen von Basispulver→Härten→Sprühen einer schwarzen Farbe→Härten→Bearbeiten einer gedrehten glänzenden Oberfläche→Vorbehandeln→Trocknen→Sprühen von transparentem Pulver→Härten→Sprühen einer farbigen Zelluloidfarbe→Härten,
wobei im Prozess des Sprühens einer farbigen Zelluloidfarbe eine Rotationsbecher-Sprühpistole zum Sprühen verwendet wird, die Drehzahl 25000 U/min beträgt, das Formiergas 2~3 bar beträgt und der Farbausstoßdruck 4~5 bar beträgt, wodurch sichergestellt wird, dass die farbige Zelluloidfarbe gleichmäßig und vollständig auf die Oberfläche der Nabe gesprüht wird; und
wobei im Prozess des Härtens der farbigen Zelluloidfarbe die Temperatur des Werkstücks 10~15 Minuten lang auf 150 °C geregelt wird, so dass die farbige Zelluloidfarbe eine bessere Flexibilität und Beschichtungshaftung aufweist.

2. Verfahren nach Anspruch 1, wobei (1) im Prozess des Sprühens der Basispulver eine elektrostatische Sprühpistole zum Sprühen verwendet wird, die Spannung auf 60~80 KV geregelt wird und die Pulverausstoß auf 10~15 g/s geregelt wird, wodurch eine hervorragende Haftung zwischen Beschichtungen sichergestellt wird; und/oder
(2) im Prozess des Härtens der Basispulver die Oberflächentemperatur eines Werkstücks 8~12 Minuten lang auf 180 °C geregelt wird, so dass das Pulver eine gewisse Flexibilität und eine bessere Beschichtungshaftung behält.

3. Verfahren nach Anspruch 1 oder 2, wobei im Prozess des Sprühens einer schwarzen Farbe eine Luftsprühpistole zum Sprühen verwendet wird, der Luftausstoß auf 50~100 cc/min geregelt wird und der Zerstäubungssektordruck 2~3 bar beträgt, wodurch sichergestellt wird, dass die schwarze Farbe gleichmäßig und vollständig auf die Oberfläche der Nabe gesprüht wird; und/oder
im Prozess des Härtens der schwarzen Farbe die Temperatur des Werkstücks 10~15 Minuten lang auf 150 °C geregelt wird, so dass die schwarze Farbe eine gute Flexibilität und Beschichtungshaftung aufweist.

4. Verfahren nach einem der Ansprüche 1 bis 3, wobei im Prozess der Bearbeitung einer gedrehten glänzenden Oberfläche die Drehzahl S auf 1200 U/min geregelt wird und die Vorschubgeschwindigkeit F 0,2 mm/U beträgt.

5. Verfahren nach einem der Ansprüche 1 bis 4, wobei im Prozess des Sprühens der transparenten Pulver die elektrostatische Sprühpistole zum Sprühen verwendet wird, die Spannung auf 60~80 KV geregelt wird und die Pulverausstoß auf 10~15 g/s geregelt wird, wodurch eine hervorragende Haftung zwischen Beschichtungen sichergestellt wird; und/oder
im Prozess des Härtens der transparenten Pulver die Oberflächentemperatur des Werkstücks 10~15 Minuten lang auf 177 °C geregelt wird, so dass das Pulver eine gewisse Flexibilität und eine bessere Haftung der Beschichtung behält.

6. Verfahren nach einem der Ansprüche 1 bis 5, wobei
im Prozess des Sprühens der Basispulver eine elektrostatische Sprühpistole zum Sprühen verwendet wird, die Spannung auf 60 KV geregelt wird und die Pulverausstoß auf 10 g/s geregelt wird, wodurch eine hervorragende Haftung zwischen Beschichtungen sichergestellt wird;
im Prozess des Härtens der Basispulver die Oberflächentemperatur eines Werkstücks 8 Minuten lang auf 180 °C geregelt wird, so dass das Pulver eine gewisse Flexibilität und eine bessere Beschichtungshaftung behält;
im Prozess des Sprühens einer schwarzen Farbe eine Luftsprühpistole zum Sprühen verwendet wird, der Luftausstoß auf 50 cc/min geregelt wird und der Zerstäubungssektordruck 2 bar beträgt, wodurch sichergestellt wird, dass die schwarze Farbe gleichmäßig und vollständig auf die Oberfläche der Nabe gesprüht wird;
im Prozess des Härtens der schwarzen Farbe die Temperatur des Werkstücks 10 Minuten lang auf 150 °C geregelt wird, so dass die schwarze Farbe eine gute Flexibilität und Beschichtungshaftung aufweist;
im Prozess der Bearbeitung einer gedrehten glänzenden Oberfläche die Drehzahl S auf 1200 U/min geregelt wird und die Vorschubgeschwindigkeit F 0,2 mm/U beträgt;
im Prozess des Sprühens der transparenten Pulver die elektrostatische Sprühpistole zum Sprühen verwendet wird, die Spannung auf 60 KV geregelt wird und die Pulverausstoß auf 10 g/s geregelt wird, wodurch eine hervorragende Haftung zwischen Beschichtungen sichergestellt wird;
im Prozess des Härtens der transparenten Pulver die Oberflächentemperatur des Werkstücks 8 Minuten lang auf 177 °C geregelt wird, so dass das Pulver eine gewisse Flexibilität und eine bessere Haftung der Beschichtung behält;
im Prozess des Sprühens einer farbigen Zelluloidfarbe eine Rotationsbecher-Sprühpistole zum Sprühen verwendet wird, die Drehzahl 25000 U/min beträgt; und
wobei im Prozess des Härtens der farbigen Zelluloidfarbe die Temperatur des Werkstücks 10 Minuten lang auf 150 °C geregelt wird, so dass die farbige Zelluloidfarbe eine bessere Flexibilität und Beschichtungshaftung aufweist.

7. Verfahren nach einem der Ansprüche 1 bis 5, wobei
im Prozess des Sprühens der Basispulver eine elektrostatische Sprühpistole zum Sprühen verwendet wird, die Spannung auf 70 KV geregelt wird und die Pulverausstoß auf 12 g/s geregelt wird, wodurch eine hervorragende Haftung zwischen Beschichtungen sichergestellt wird;
im Prozess des Härtens der Basispulver die Oberflächentemperatur eines Werkstücks 10 Minuten lang auf 180 °C geregelt wird, so dass das Pulver eine gewisse Flexibilität und eine bessere Beschichtungshaftung behält;
im Prozess des Sprühens einer schwarzen Farbe eine Luftsprühpistole zum Sprühen verwendet wird, der Luftausstoß auf 80 cc/min geregelt wird und der Zerstäubungssektordruck 2.5 bar beträgt, wodurch sichergestellt wird, dass die schwarze Farbe gleichmäßig und vollständig auf die Oberfläche der Nabe gesprüht wird;
im Prozess des Härtens der schwarzen Farbe die Temperatur des Werkstücks 12 Minuten lang auf 150 °C geregelt wird, so dass die schwarze Farbe eine gute Flexibilität und Beschichtungshaftung aufweist;
im Prozess der Bearbeitung einer gedrehten glänzenden Oberfläche die Drehzahl S auf 1200 U/min geregelt wird und die Vorschubgeschwindigkeit F 0,2 mm/U beträgt;
im Prozess des Sprühens der transparenten Pulver die elektrostatische Sprühpistole zum Sprühen verwendet wird, die Spannung auf 70 KV geregelt wird und die Pulverausstoß auf 12 g/s geregelt wird, wodurch eine hervorragende Haftung zwischen Beschichtungen sichergestellt wird;
im Prozess des Härtens der transparenten Pulver die Oberflächentemperatur des Werkstücks 12 Minuten lang auf 177 °C geregelt wird, so dass das Pulver eine gewisse Flexibilität und eine bessere Haftung der Beschichtung behält;
im Prozess des Sprühens einer farbigen Zelluloidfarbe eine Rotationsbecher-Sprühpistole zum Sprühen verwendet wird, die Drehzahl 25000 U/min beträgt, das Formiergas 2.5 bar beträgt und der Farbausstoßdruck 4.5 bar beträgt, wodurch sichergestellt wird, dass die farbige Zelluloidfarbe gleichmäßig und vollständig auf die Oberfläche der Nabe gesprüht wird; und
wobei im Prozess des Härtens der farbigen Zelluloidfarbe die Temperatur des Werkstücks 12 Minuten lang auf 150 °C geregelt wird, so dass die farbige Zelluloidfarbe eine bessere Flexibilität und Beschichtungshaftung aufweist.

8. Verfahren nach einem der Ansprüche 1 bis 5, wobei
im Prozess des Sprühens der Basispulver eine elektrostatische Sprühpistole zum Sprühen verwendet wird, die Spannung auf 80 KV geregelt wird und die Pulverausstoß auf 15 g/s geregelt wird, wodurch eine hervorragende Haftung zwischen Beschichtungen sichergestellt wird;
im Prozess des Härtens der Basispulver die Oberflächentemperatur eines Werkstücks 12 Minuten lang auf 180 °C geregelt wird, so dass das Pulver eine gewisse Flexibilität und eine bessere Beschichtungshaftung behält;
im Prozess des Sprühens einer schwarzen Farbe eine Luftsprühpistole zum Sprühen verwendet wird, der Luftausstoß auf 100 cc/min geregelt wird und der Zerstäubungssektordruck 3 bar beträgt, wodurch sichergestellt wird, dass die schwarze Farbe gleichmäßig und vollständig auf die Oberfläche der Nabe gesprüht wird;
im Prozess des Härtens der schwarzen Farbe die Temperatur des Werkstücks 15 Minuten lang auf 150 °C geregelt wird, so dass die schwarze Farbe eine gute Flexibilität und Beschichtungshaftung aufweist;
im Prozess der Bearbeitung einer gedrehten glänzenden Oberfläche die Drehzahl S auf 1200 U/min geregelt wird und die Vorschubgeschwindigkeit F 0,2 mm/U beträgt;
im Prozess des Sprühens der transparenten Pulver die elektrostatische Sprühpistole zum Sprühen verwendet wird, die Spannung auf 80 KV geregelt wird und die Pulverausstoß auf 15 g/s geregelt wird, wodurch eine hervorragende Haftung zwischen Beschichtungen sichergestellt wird;
im Prozess des Härtens der transparenten Pulver die Oberflächentemperatur des Werkstücks 15 Minuten lang auf 177 °C geregelt wird, so dass das Pulver eine gewisse Flexibilität und eine bessere Haftung der Beschichtung behält;
im Prozess des Sprühens einer farbigen Zelluloidfarbe eine Rotationsbecher-Sprühpistole zum Sprühen verwendet wird, die Drehzahl 25000 U/min beträgt, das Formiergas 3 bar beträgt und der Farbausstoßdruck 5 bar beträgt, wodurch sichergestellt wird, dass die farbige Zelluloidfarbe gleichmäßig und vollständig auf die Oberfläche der Nabe gesprüht wird; und
wobei im Prozess des Härtens der farbigen Zelluloidfarbe die Temperatur des Werkstücks 15 Minuten lang auf 150 °C geregelt wird, so dass die farbige Zelluloidfarbe eine bessere Flexibilität und Beschichtungshaftung aufweist.

## Revendications

1. Un procédé de pulvérisation à registre de couleur d'un moyeu, comprenant : après qu'une peinture noire a été pulvérisée sur la surface du moyeu, usiner l'une surface brillante tournée, puis pulvériser le moyeu avec une peinture celluloïd de couleur,
dans lequel le procédé comprend les étapes de : prétraitement→séchage→pulvérisation d'une poudre de base→durcissement→pulvérisation d'une peinture noire→durcissement→usinage d'une surface brillante tournée→prétraitement→séchage→pulvérisation d'une poudre transparente→durcissement→pulvérisation d'une peinture celluloïd de couleur→durcissement,
dans lequel, dans le processus de pulvérisation d'une peinture celluloïd de couleur, un pistolet pulvérisateur à coupelle rotative est adopté pour la pulvérisation, la vitesse de rotation est de 25000 R/min, le gaz de formation est de 2 à 3 bars et la pression de sortie de la peinture est de 4 à 5 bars, garantissant ainsi que la peinture celluloïd de couleur est uniformément et entièrement pulvérisée sur la surface du moyeu ; et
dans lequel, dans le processus de durcissement de la peinture celluloïd de couleur, la température de la pièce est contrôlée à 150°C pendant 10 à 15 min, de sorte que la peinture celluloïd de couleur ait une meilleure flexibilité et une meilleure adhérence du revêtement.

2. Le procédé selon la revendication 1, dans lequel (1) dans le processus de pulvérisation de poudre de base, un pistolet de pulvérisation électrostatique est adopté pour la pulvérisation, la tension est contrôlée à 60~80 KV et la sortie de poudre est contrôlée à 10~15 g/s, assurant ainsi une excellente adhérence entre les revêtements ; et/ou
(2) dans le processus de durcissement de la poudre de base, la température de surface d'une pièce est contrôlée à 180 ° C pendant 8 ~ 12 min, de sorte que la poudre conserve une certaine flexibilité et une meilleure adhérence du revêtement.

3. Le procédé selon la revendication 1 ou 2, dans lequel, dans le processus de pulvérisation d'une peinture noire, un pistolet pulvérisateur à air est adopté pour la pulvérisation, la sortie d'air est contrôlée à 50~100 cc/min, et la pression du secteur d'atomisation est de 2~3 bar, garantissant ainsi que la peinture noire est uniformément et entièrement pulvérisée sur la surface du moyeu ; et/ou
dans le processus de durcissement de la peinture noire, la température de la pièce est contrôlée à 150 ° C pendant 10 ~ 15 min, de sorte que la peinture noire ait une bonne flexibilité et une bonne adhérence du revêtement.

4. Le procédé selon l'une des revendications 1 à 3, dans lequel, dans le processus d'usinage d'une surface brillante tournée, la vitesse de rotation S est contrôlée à 1200 rpm, et la vitesse d'alimentation F est de 0,2 mm/r.

5. Le procédé selon l'une des revendications 1 à 4, dans lequel, dans le processus de pulvérisation de poudre transparente, le pistolet de pulvérisation électrostatique est adopté pour la pulvérisation, la tension est contrôlée à 60 ~ 80 KV, et la sortie de poudre est contrôlée à 10 ~ 15 g /s, assurant ainsi une excellente adhérence entre les revêtements ; et/ou
dans le processus de durcissement de la poudre transparente, la température de surface de la pièce est contrôlée à 177 ° C pendant 10 ~ 15 min, de sorte que la poudre conserve une certaine flexibilité et une meilleure adhérence du revêtement.

6. Le procédé selon l'une des revendications 1 à 5, dans lequel,
dans le processus de pulvérisation de poudre de base, un pistolet de pulvérisation électrostatique est adopté pour la pulvérisation, la tension est contrôlée à 60 KV et le sortie de poudre est contrôlé à 10 g/s, assurant ainsi une excellente adhérence entre les revêtements ;
dans le processus de durcissement de la poudre de base, la température de surface d'une pièce est contrôlée à 180°C pendant 8 min, de sorte que la poudre conserve une certaine flexibilité et une meilleure adhérence du revêtement ;
dans le processus de pulvérisation d'une peinture noire, un pistolet pulvérisateur à air est adopté pour la pulvérisation, la sortie d'air est contrôlé à 50 cc/min et la pression du secteur d'atomisation est de 2 bars, garantissant ainsi que la peinture noire est uniformément et entièrement pulvérisée sur la surface du moyeu ;
dans le processus de durcissement de la peinture noire, la température de la pièce est contrôlée à 150°C pendant 10 min, de sorte que la peinture noire ait une bonne flexibilité et une bonne adhérence du revêtement ;
dans le processus d'usinage d'une surface brillante tournée, la vitesse de rotation S est contrôlée à 1200 rpm, et la vitesse d'alimentation F est de 0,2 mm/r ;
dans le processus de pulvérisation de poudre transparente, le pistolet de pulvérisation électrostatique est adopté pour la pulvérisation, la tension est contrôlée à 60 KV et la sortie de poudre est contrôlée à 10 g/s, assurant ainsi une excellente adhérence entre les revêtements ;
dans le processus de durcissement de la poudre transparente, la température de surface de la pièce est contrôlée à 177°C pendant 8 min, de sorte que la poudre conserve une certaine flexibilité et une meilleure adhérence du revêtement ;
dans le processus de pulvérisation d'une peinture celluloïd de couleur, un pistolet pulvérisateur à coupelle rotative est adopté pour la pulvérisation, et la vitesse de rotation est de25000 R/min ; et
dans le processus de durcissement de la peinture celluloïd de couleur, la température de la pièce est contrôlée à 150 ° C pendant 10 min, de sorte que la peinture celluloïd de couleur ait une meilleure flexibilité et une meilleure adhérence du revêtement.

7. Le procédé selon l'une des revendications 1 à 5, dans lequel,
dans le processus de pulvérisation de poudre de base, un pistolet de pulvérisation électrostatique est adopté pour la pulvérisation, la tension est contrôlée à 70 KV et le sortie de poudre est contrôlé à 12 g/s, assurant ainsi une excellente adhérence entre les revêtements ;
dans le processus de durcissement de la poudre de base, la température de surface d'une pièce est contrôlée à 180°C pendant 10 min, de sorte que la poudre conserve une certaine flexibilité et une meilleure adhérence du revêtement ;
dans le processus de pulvérisation d'une peinture noire, un pistolet pulvérisateur à air est adopté pour la pulvérisation, la sortie d'air est contrôlé à 80 cc/min et la pression du secteur d'atomisation est de 2,5 bars, garantissant ainsi que la peinture noire est uniformément et entièrement pulvérisée sur la surface du moyeu ;
dans le processus de durcissement de la peinture noire, la température de la pièce est contrôlée à 150°C pendant 12 min, de sorte que la peinture noire ait une bonne flexibilité et une bonne adhérence du revêtement ;
dans le processus d'usinage d'une surface brillante tournée, la vitesse de rotation S est contrôlée à 1200 rpm, et la vitesse d'alimentation F est de 0,2 mm/r ;
dans le processus de pulvérisation de poudre transparente, le pistolet de pulvérisation électrostatique est adopté pour la pulvérisation, la tension est contrôlée à 70 KV et la sortie de poudre est contrôlée à 12 g/s, assurant ainsi une excellente adhérence entre les revêtements ;
dans le processus de durcissement de la poudre transparente, la température de surface de la pièce est contrôlée à 177°C pendant 12 min, de sorte que la poudre conserve une certaine flexibilité et une meilleure adhérence du revêtement ;
dans le processus de pulvérisation d'une peinture celluloïd de couleur, un pistolet pulvérisateur à coupelle rotative est adopté pour la pulvérisation, et la vitesse de rotation est de 25000 R/min, le gaz de formation est de 2.5 bars et la pression de sortie de la peinture est de 4.5 bars, garantissant ainsi que la peinture celluloïd de couleur est uniformément et entièrement pulvérisée sur la surface du moyeu; et
dans le processus de durcissement de la peinture celluloïd de couleur, la température de la pièce est contrôlée à 150 ° C pendant 12 min, de sorte que la peinture celluloïd de couleur ait une meilleure flexibilité et une meilleure adhérence du revêtement.

8. Le procédé selon l'une des revendications 1 à 5, dans lequel,
dans le processus de pulvérisation de poudre de base, un pistolet de pulvérisation électrostatique est adopté pour la pulvérisation, la tension est contrôlée à 80 KV et le sortie de poudre est contrôlé à 15 g/s, assurant ainsi une excellente adhérence entre les revêtements ;
dans le processus de durcissement de la poudre de base, la température de surface d'une pièce est contrôlée à 180°C pendant 12 min, de sorte que la poudre conserve une certaine flexibilité et une meilleure adhérence du revêtement ;
dans le processus de pulvérisation d'une peinture noire, un pistolet pulvérisateur à air est adopté pour la pulvérisation, la sortie d'air est contrôlé à 100 cc/min et la pression du secteur d'atomisation est de 3 bars, garantissant ainsi que la peinture noire est uniformément et entièrement pulvérisée sur la surface du moyeu ;
dans le processus de durcissement de la peinture noire, la température de la pièce est contrôlée à 150°C pendant 15 min, de sorte que la peinture noire ait une bonne flexibilité et une bonne adhérence du revêtement ;
dans le processus d'usinage d'une surface brillante tournée, la vitesse de rotation S est contrôlée à 1200 rpm, et la vitesse d'alimentation F est de 0,2 mm/r ;
dans le processus de pulvérisation de poudre transparente, le pistolet de pulvérisation électrostatique est adopté pour la pulvérisation, la tension est contrôlée à 80 KV et la sortie de poudre est contrôlée à 15 g/s, assurant ainsi une excellente adhérence entre les revêtements ;
dans le processus de durcissement de la poudre transparente, la température de surface de la pièce est contrôlée à 177°C pendant 15 min, de sorte que la poudre conserve une certaine flexibilité et une meilleure adhérence du revêtement ;
dans le processus de pulvérisation d'une peinture celluloïd de couleur, un pistolet pulvérisateur à coupelle rotative est adopté pour la pulvérisation, la vitesse de rotation est de 25000 R/min, le gaz de formage est de 3 bars et la pression de sortie de peinture est de 5 bars, garantissant ainsi que la couleur la peinture celluloïd est uniformément et entièrement pulvérisée sur la surface du moyeu ; et
dans le processus de durcissement de la peinture celluloïd de couleur, la température de la pièce est contrôlée à 150 ° C pendant 15 min, de sorte que la peinture celluloïd de couleur ait une meilleure flexibilité et une meilleure adhérence du revêtement.
